

## UNITED STATES PATENT OFFICE.

JOHN A. GANN, OF MIDLAND, MICHIGAN, ASSIGNOR TO THE DOW CHEMICAL COMPANY, OF MIDLAND, MICHIGAN, A CORPORATION OF MICHIGAN.

## TREATMENT OF MAGNESIUM-BASE ALLOYS.

No Drawing.

Application filed March 29, 1927. Serial No. 179,402.

In my co-pending application filed November 28, 1921, Ser. No. 518,142, I describe an improvement in the art of making alloy articles having magnesium as the principal 5 ingredient and containing one or more metals capable of dissolving in solid magnesium in larger amounts than are found in solution in the alloy as cast, such improvement consisting in subjecting such an article to a 10 heat treatment at high temperature but below the melting temperature of the most fusible constituent of the alloy. The result of the aforesaid treatment is to cause increased solution of the other metal or metals 15 in the solid magnesium, this being accompanied by a marked increase in the strength and/or plasticity of the article as well as in the improvement thereof in other of its physical characteristics. The increase in 20 plasticity thus obtained in light metal alloy articles of the class in question is of particular importance where it is desired subsequently to subject the article to plastic deformation, such for example as a forging, 25 drawing, rolling or extruding operation. The articles thus treated are also found to be rendered susceptible to further improvement in certain physical qualities by aging at regulated temperatures.

30 The improvements herein claimed relate to certain specific aspects of the process and resultant product described in my aforesaid application, it being noted that other such specific aspects are separately presented in 35 my co-pending application filed January 13, 1927, Ser. No. 161,029. It has been found, in other words, that specifically different results may be obtained, depending upon the 40 constitution of the alloy that is subjected to the aforesaid heat treatment, and while a wider field of use will probably be found with magnesium-aluminum alloys, other binary as well as ternary and more complex 45 magnesium alloys are susceptible to marked improvement by treatment in the fashion described.

Having regard to the accomplishment of the foregoing and related ends, the invention then consists of the steps hereinafter 50 fully described and particularly pointed out in the claims, the following description setting forth but one of the various ways in

which the principle of the invention may be used.

In my co-pending application first referred to above, more particular emphasis is placed on the improved results obtained by my method of regulated heat treatment in the case of a magnesium-aluminum alloy, the one selected by way of example containing from 6 to 8 per cent aluminum. However, reference is also made in said application, as well as in my second co-pending application, to the effect of such heat treatment on a ternary or more complex magnesium alloy, in which at least part of the added metals form eutectics with the magnesium and said eutectics have different melting points and vary as to the ease with which they dissolve in the magnesium to form solid solutions whereby one or more of the added metals are caused to be present both as solid solution and eutectic, while the other or others are present either as solid solution or eutectic. As an example of the latter, magnesium-aluminum-zinc-copper-cadmium alloys are cited in which the heat treatment may be such that aluminum and zinc are present as both solid solutions and eutectic, while the copper is present as eutectic and the cadmium is completely in solid solution.

A typical alloy of the kind in question is one containing approximately 8.5 per cent of aluminum, 2 per cent of copper and 1 per cent of zinc, with or without a corresponding small percentage of cadmium, the balance being magnesium. Such an alloy as cast will contain an eutectic structure formed by each of the three first-named alloying ingredients with the magnesium, in addition to a certain amount of solid solution formed by the aluminum and zinc with the magnesium. The copper, on the contrary, will not form such solid solution and this remains true even after heat treatment of the alloy, while, on the contrary, all of the cadmium immediately goes into such solution and so remains.

The melting point of the Mg-Al eutectic is 100 824 degrees F., while the Mg-Zn eutectic melts at 650 degrees F. Accordingly, in carrying out my method of regulated heat treatment in the case of such an alloy, it

is initially heated to a temperature somewhat lower than the melting point of such last mentioned eutectic, e. g., at 645 degrees F., until such time as the zinc is found entirely to have gone into solid solution with the magnesium. Thereupon the temperature may be raised to approximately 820 degrees F. and the heat treatment continued, if desired, until all of the aluminum has likewise dissolved with the magnesium, or such heat treatment may be stopped short of the point of such complete solution of the aluminum so as to leave a residual Mg-Al eutectic structure. In any event the alloy after heat treatment will retain, as above explained, the Mg-Cu eutectic structure which does not dissolve at all, although the prescribed heat treatment may cause some rearrangement of this eutectic with attendant relief of casting strains that may be present in the article. Similarly, where cadmium is present, such heat treatment will insure a more uniform distribution thereof in solution by eliminating cored crystals which otherwise may be present.

It will be understood, of course, that a lower temperature may be employed in each of the foregoing stages of the heat treatment, provided the latter be sufficiently prolonged. The change in the micro-structure of the alloy serves very definitely to establish the completion of the heat treatment, whether conducted at a lower temperature for such longer period or at a higher temperature approximating the maximum permissible temperature as determined by the melting point of the more fusible eutectic present in the alloy.

The term "eutectic", as herein used, it will be understood, includes not only the well-known ordinary eutectics with their more or less characteristic lamellar or globular structure, but also individual more or less well-defined metallic or intermetallic crystals which so often occur with relatively small percentages of added constituents.

Other modes of applying the principle of my invention may be employed instead of the one explained, change being made as regards the composition and method herein disclosed, provided the ingredients or steps stated by any of the following claims or the equivalent of such stated ingredients or steps be employed.

I therefore particularly point out and distinctly claim as my invention:

1. In the art of making light metal alloy articles wherein magnesium is the predominant constituent, the alloy containing as minor constituents two other metals capable of forming eutectics differing as to their melting points, and also as to ease with which they dissolve in the magnesium to form a solid solution, the steps which consist in heating such an article at a high tem-

perature but below the melting point of the more fusible eutectic, to cause substantially complete solution thereof, and then heating such article at a higher temperature but below the melting point of the less fusible eutectic to cause increased solution thereof. 70

2. In the art of making light metal alloy articles wherein magnesium is the predominant constituent, the alloy containing as minor constituents two other metals capable of forming eutectics differing as to their melting points, and also as to ease with which they dissolve in the magnesium to form a solid solution, the steps which consist in heating such an article at a high temperature but below the melting point of the more fusible eutectic, to cause substantially complete solution of the same, and then heating such article at a higher temperature but below the melting point of the less fusible eutectic to cause substantially complete solution thereof. 80

3. In the art of making light metal alloy articles wherein magnesium is the predominant constituent, the alloy containing as minor constituents two other metals capable of forming eutectics differing as to their melting points, and also as to ease with which they dissolve in the magnesium to form a solid solution, said alloy also containing as a minor constituent a metal forming a substantially insoluble eutectic with the magnesium, the steps which consist in heating such an article at a high temperature but below the melting point of the more fusible of such soluble eutectics, to cause substantially complete solution thereof, and then heating such article at a higher temperature but below the melting point of the less fusible of such soluble eutectics to cause increased solution thereof. 90

4. In the art of making light metal alloy articles wherein magnesium is the predominant constituent, the alloy containing as minor constituents two other metals capable of forming eutectics differing as to their melting points, and also as to ease with which they dissolve in the magnesium to form a solid solution, said alloy also containing as a minor constituent a metal forming a substantially insoluble eutectic with the magnesium, the steps which consist in heating such an article at a high temperature but below the melting point of the more fusible of such soluble eutectics, to cause substantially complete solution thereof, and then heating such article at a higher temperature but below the melting point of the less fusible of such soluble eutectics to cause substantially complete solution thereof. 100

5. In the art of making light metal alloy articles wherein magnesium is the predominant constituent, the alloy containing zinc and aluminum as minor constituents, 130

the step which consists in heating such an article at a high temperature, but below the melting point of the eutectic formed by the zinc to cause substantially complete solution 5 thereof.

6. In the art of making light metal alloy articles wherein magnesium is the predominant constituent, the alloy containing zinc and aluminum as minor constituents, 10 the step which consists in heating such an article at a high temperature, but below the melting point of the eutectic formed by the zinc to cause substantially complete solution thereof, and then heating such article at a 15 higher temperature but below the melting point of the eutectic formed by the aluminum to cause increased solution thereof.

7. In the art of making light metal alloy articles wherein magnesium is the predominant constituent, the alloy containing zinc and aluminum as minor constituents, the step which consists in heating such an article at a high temperature, but below the melting point of the eutectic formed by the 25 zinc to cause substantially complete solution thereof, and then heating such article at a higher temperature but below the melting point of the eutectic formed by the aluminum to cause substantially complete solution 30 thereof.

8. In the art of making light metal alloy articles wherein magnesium is the predominant constituent, the alloy containing zinc, aluminum and copper as minor constituents, 35 the step which consists in treating such an article at a high temperature, but below the melting point of the eutectic formed by the zinc, to cause substantially complete solution of the latter.

40 9. In the art of making light metal alloy articles wherein magnesium is the predominant constituent, the alloy containing zinc, aluminum and copper as minor constituents, the step which consists in treating such an 45 article at a high temperature, but below the melting point of the eutectic formed by the zinc, to cause substantially complete solution of the latter, and then heating such article at a higher temperature but below the 50 melting point of the eutectic formed by the aluminum to cause increased solution thereof.

10. In the art of making light metal alloy articles wherein magnesium is the predominant constituent, the alloy containing zinc, aluminum and copper as minor constituents, the step which consists in treating such an article at a high temperature, but below the melting point of the eutectic formed by the zinc, to cause substantially complete solution of the latter, and then heating such article at a higher temperature but below the melting point of the eutectic formed by the aluminum to cause substantially complete solution thereof.

11. As an article of manufacture, a heat treated light metal alloy article, wherein magnesium is the predominant constituent, the alloy also containing as minor constituents two other metals capable of forming 70 eutectics differing as to their melting points as also as to the ease with which they dissolve in the magnesium to form a solid solution, such treated article being characterized by having a greater amount of the more soluble constituent present in solution than in an untreated article of the same composition. 75

12. As an article of manufacture, a heat treated light metal alloy article, wherein magnesium is the predominant constituent, 80 the alloy also containing as minor constituents two other metals capable of forming eutectics differing as to their melting points as also as to the ease with which they dissolve in the magnesium to form a solid solution, such treated article being characterized by having substantially all of the more soluble constituent present in solution. 85

13. As an article of manufacture, a heat treated light metal alloy article, wherein 90 magnesium is the predominant constituent, the alloy also containing as minor constituents two other metals capable of forming eutectics differing as to their melting points as also as to the ease with which they dissolve in the magnesium to form a solid solution, such treated article being characterized by having substantially all of both such minor constituents present in solution. 95

14. As an article of manufacture, a heat 100 treated light metal alloy article, wherein magnesium is the predominant constituent, the alloy also containing zinc and aluminum as minor constituents, such treated article being characterized by having a greater 105 amount of zinc present in solution than in an untreated article of the same composition.

15. As an article of manufacture, a heat treated light metal alloy article, wherein 110 magnesium is the predominant constituent, the alloy also containing zinc and aluminum as minor constituents, such treated article being characterized by having all of the zinc present in solution. 115

16. As an article of manufacture, a heat treated light metal alloy article, wherein magnesium is the predominant constituent, the alloy also containing zinc and aluminum as minor constituents, such treated article 120 being characterized by having all of the zinc present in solution and a greater amount of aluminum thus in solution than in an untreated casting.

17. As an article of manufacture, a heat 125 treated light metal alloy article, wherein magnesium is the predominant constituent, the alloy also containing zinc, aluminum and copper as minor constituents, such treated article being characterized by hav- 130

ing all of the zinc present in solution, the copper remaining in the eutectic structure.

18. As an article of manufacture, a heat treated light metal alloy article, wherein magnesium is the predominant constituent, the alloy also containing zinc, aluminum and copper as minor constituents, such treated article being characterized by having a greater amount of zinc and aluminum present in solution than in an untreated article of the same composition, the copper remaining in the eutectic structure.

19. As an article of manufacture, a heat treated light metal alloy article, wherein magnesium is the predominant constituent, the alloy also containing zinc, aluminum and copper as minor constituents, such treated article being characterized by having substantially all of the zinc and aluminum present in solution, the copper remaining in a eutectic structure.

Signed by me this 19th day of January, 1927.

JOHN A. GANN.